

# UNITED STATES PATENT OFFICE.

GEORGE W. PRIEST, OF WILMINGTON, DELAWARE, ASSIGNOR TO E. I. DU PONT DE NEMOURS AND COMPANY, OF WILMINGTON, DELAWARE, A CORPORATION OF DELAWARE.

## METHOD FOR PRODUCING LINOLEUM AND PRODUCT THEREOF.

1,334,049.

Specification of Letters Patent. Patented Mar. 16, 1920.

No Drawing.

Application filed August 8, 1917. Serial No. 185,015.

*To all whom it may concern:*

Be it known that I, GEORGE W. PRIEST, of Wilmington, in the county of New Castle, and in the State of Delaware, have invented 5 a certain new and useful Improvement in Methods for Producing Linoleum and Product Thereof, and do hereby declare that the following is a full, clear, and exact description thereof.

10 My invention relates to a new linoleum and a process of making the same.

The object of my invention is to provide a linoleum article containing polymerized Chinese wood oil or tung oil and a polymerized product of the coumarone or indene group of compounds combined in an advantageous manner.

Further objects of my invention will appear from the detailed description thereof 20 contained hereinafter.

I have found that when previously polymerized Chinese wood oil or tung oil is ground together in any suitable machine, as for example a machine containing friction 25 rolls, with a polymerized product of the coumarone or indene group of compounds at a temperature of 100° C. or below a material is obtained which has different characteristics as to its consistency, combining 30 qualities, solubility, etc. which make it more useful as a cement than in the case where the polymerized product of the coumarone or indene group of compounds is added to the Chinese wood oil when heated 35 to above 100° C.

While my invention is capable of being carried out in many different ways, I shall describe only one example thereof herein-after.

40 In order to carry out my process I may for example heat two parts of Chinese wood oil or tung oil to 265° C., so as to polymerize the same and produce a jelly-like material. The material thus obtained is allowed to cool and I then mix therewith one 45 part of a polymerized product of the coumarone or indene group of compounds and grind the same together at a temperature of 100 C. or below thus producing a composition which is elastic, adhesive, coherent 50 and light in color.

This composition may be used for lino-

leum cement by mixing with suitable proportions of pigment, ground cork, or woodmeal, as for example—

55

|                                      |           |
|--------------------------------------|-----------|
| Tung oil coumarone resin composition | 50 parts. |
| Pigment                              | 20 "      |
| Ground cork or woodmeal              | 50 " 60   |

and applying to a fabric by means of pressure. The material may also be used for cementing materials of other kinds together, and on fabrics of all kinds.

While I have described my invention 65 above in detail, I wish it to be understood that many changes may be made therein without departing from the spirit of the same.

What I claim is:—

70

1. The process which comprises mixing together an oil and a polymerized product of the coumarone or indene group of compounds at a temperature not above 100° C. and so applying the mixture to a fabric 75 layer as to cause it to adhere thereto.

2. The process which comprises mixing together an oil and a polymerized product of the coumarone or indene group of compounds at a temperature not above 100° C., 80 and so applying the mixture together with ground cork to a fabric layer as to cause it to adhere thereto.

3. The process which comprises mixing together polymerized Chinese wood oil and 85 a polymerized product of the coumarone or indene group of compounds at a temperature not above 100° C., and so applying the mixture to a fabric layer as to cause it to 90 adhere thereto.

4. The process which comprises mixing together polymerized Chinese wood oil and a polymerized product of the coumarone or indene group of compounds at a temperature not above 100° C., and so applying the 95 mixture together with ground cork to a fabric layer as to cause it to adhere thereto.

5. An article of manufacture comprising an oil mixed with a polymerized product of the coumarone or indene group of compounds, and a fabric layer carrying the same. 100

6. An article of manufacture comprising polymerized Chinese wood oil mixed with a

polymerized product of the coumarone or indene group of compounds, and a fabric layer carrying the same.

7. An article of manufacture comprising  
5 polymerized Chinese wood oil mixed with a polymerized product of the coumarone or indene group of compounds and ground cork mixed therewith, and a fabric layer carrying the same.

- 10 8. An article of manufacture comprising

a thickened oil mixed with a polymerized product of the coumarone or indene group of compounds, and a fabric layer carrying the same.

In testimony that I claim the foregoing 15  
I have hereunto set my hand.

GEORGE W. PRIEST.

Witnesses:

P. STRICKLAND,  
H. J. HAWKE, JR.